

## UNITED STATES PATENT OFFICE

2,383,976

## ALLOYS

Robert H. Leach, Fairfield, Conn., assignor to  
Handy & Harman, New York, N. Y., a corpora-  
tion of New York

No Drawing. Application September 26, 1942,  
Serial No. 459,833

## 4 Claims. (Cl. 75—173)

This invention relates to alloys to be used for brazing and welding purposes and is concerned more particularly with novel quaternary alloys of silver, copper, cadmium, and zinc. The new alloys flow freely at relatively low temperatures and are of such physical characteristics that they may be fabricated into forms convenient for use and joints made with them have the desired physical strength.

Quaternary brazing alloys of silver, copper, cadmium, and zinc are not broadly new and in my Patent No. 1,899,701 issued February 28, 1933, I described alloys of that type that have proven highly satisfactory for commercial purposes and have been sold in large quantities. The patented alloys flow freely at 1175° F. or less and have such malleability, ductility, and strength as to be readily fabricated into sheet and wire and to make strong joints. In those alloys, the silver content ranges from about 48 to 52% and the preferred commercial form contains about 50% of silver.

As a result of further investigation of the properties of the quaternary alloys of silver, copper, cadmium, and zinc, I have found that the optimum characteristics of such alloys can be obtained provided certain definite relationships among the several metals are maintained. If those relationships are observed, the alloys will have the desired qualities of low flow point, malleability, ductility, and strength, and may contain a less amount of silver than that employed in the alloys of the patent above mentioned. With the recent increases in the price of silver, the reduction of the silver content without any considerable impairment of the desirable characteristics of the alloys is of considerable importance, particularly to users engaged in manufacture on a large scale.

In the new alloys, the silver content ranges from about 44% to about 47½% and the ratio of silver to copper varies between about 2.6 and about 3.5 and the ratio of zinc to cadmium varies between about 0.9 and about 1.2.

In my Reissue Patent No. 20,638, dated January 25, 1938, I stated that the presence of zinc or cadmium or both has a bearing on the melting point of quaternary alloys, in which they are present with silver and copper, and explained that, in general, the higher the proportions of zinc or cadmium or both, the lower the melting point. I also disclosed that it is not desirable to employ an aggregate amount of zinc and cadmium in excess of about 40% and that, for most purposes, a less amount was to be preferred. In the new alloys,

to the zinc and cadmium content is followed and the total amount of zinc and cadmium is kept below about 40%.

A specific example of the new alloys may have the following approximate analysis:

## Example No. 1

|         | Per cent |
|---------|----------|
| Silver  | 45.5     |
| Copper  | 16.5     |
| Zinc    | 18.0     |
| Cadmium | 20.0     |

Alloys of the above composition flow freely at approximately 1160° F. and can be fabricated into sheet and wire. A reduction in the total amount of zinc and cadmium gives greater malleability and ductility and the alloy flows freely at about the same temperature as before. Such an alloy may be of the following approximate analysis:

## Example No. 2

|         | Per cent |
|---------|----------|
| Silver  | 47.5     |
| Copper  | 15.8     |
| Zinc    | 18.4     |
| Cadmium | 18.3     |

In the alloys of Examples Nos. 1 and 2, the silver to copper ratios are, respectively, about 2.8 and 3 and the zinc to cadmium ratios are, respectively, 0.9 and 1. If the silver content and the aggregate amount of zinc and cadmium are kept within the limits above specified and the silver-copper ratio is increased to about 3.5 and the zinc-cadmium ratio increased to about 1.2, the alloy will again flow freely at temperatures of about 1150° F. to 1160° F. An example of such an alloy is of the following approximate analysis:

## Example No. 3

|         | Per cent |
|---------|----------|
| Silver  | 47.5     |
| Copper  | 13.5     |
| Zinc    | 21.0     |
| Cadmium | 18.0     |

Alloys of the invention can be used for general brazing and welding purposes and, since they flow freely at the relatively low temperatures of about 1150° F. to about 1160° F., they are applicable for many purposes for which alloys of higher flow point cannot be used because of the liability of damage being done to the objects to be joined on exposure to high temperatures. The new alloys have satisfactory physical characteristics, as

makes their use advantageous in operations in which cost is of major importance.

I claim:

1. An alloy which consists of silver ranging from about 44% to about 47½%, copper in an amount such that the ratio of silver to copper varies between about 2.6 and about 3.5, and zinc and cadmium in an aggregate amount not exceeding about 40%, with the zinc to cadmium ratio varying from about 0.9 to about 1.2.

2. An alloy which consists of about 45.5% silver, about 16.5 copper, about 18% zinc, and about 20% cadmium.

3. An alloy which consists of about 47.5% silver, about 15.8% copper, about 18.4% zinc, and about 18.3% cadmium.

4. An alloy which consists of about 47.5% silver, about 13.5% copper, about 21% zinc, and about 18% cadmium.

ROBERT H. LEACH.